

## UNITED STATES PATENT OFFICE

2,298,557

## MINEEAL OIL COMPOSITION

Everett W. Fuller, Woodbury, N. J., assignor to  
Socony-Vacuum Oil Company, Incorporated,  
New York, N. Y., a corporation of New York

No Drawing. Application September 25, 1941,  
Serial No. 412,285

18 Claims. (Cl. 252—50)

This invention has to do with the stabilization of viscous mineral oil fractions against the deleterious effects of oxidation by the use of inhibitors of oxidation or, as more commonly designated, "oxidation-inhibitors" or "anti-oxidants." More specifically, the present invention relates to the improvement or stabilization of such mineral oil fractions by the use of a novel class of reaction products, which when admixed with viscous mineral oils in minor proportions will prevent or retard undesirable changes taking place in the oils.

To those familiar with the art it is well known that substantially all of the various mineral oil fractions are susceptible to oxidation. Such susceptibility to oxidation varies with the type and degree of refinement to which the oil has been subjected and with the conditions under which it is used or tested. Thus, the degree to which products of oxidation are formed in an oil fraction is a measure of the extent of removal of the various unstable constituents by refining operations and of the conditions of use of the oil fraction.

A highly refined viscous oil, for example, is one that has been refined by treatment with fuming sulfuric acid or with large quantities of concentrated sulfuric acid, or other means or combinations such as  $AlCl_3$ , solvents, and acids. When subjected to oxidizing conditions, such an oil tends to form relatively large amounts of acidic constituents. The presence of catalytic materials such as copper does not appear to affect appreciably the oxidation of highly refined oils, and such oils are less susceptible to the formation of colored bodies or of insoluble sludge. For most applications of these oils, however, it is desirable that acidic bodies be absent, or that no increase in acidic bodies take place under conditions of use. Acidic bodies are corrosive to metals and therefore reduce the useful life of the oils as lubricants or for other purposes for which they come in contact with metals. Similarly, acidic bodies are injurious in textile lubricants and in spray oils. When the oils are used for insulation or cooling in electrical equipment such as transformers or capacitors, an increase in acidic bodies tends to lower the dielectric strength of the oil and has other undesirable harmful effects.

Oils that have been refined by treatment with only moderate amounts of sulfuric acid or other refining agents are designated as moderately re-

fined oils. Such oils have a tendency to form relatively small amounts of acidic oxidation products as compared with highly refined oils but depreciate in color and form substantial amounts of sludge. Metal catalysts such as copper materially accelerate deterioration of these oils. The principal objection to these oils is their tendency to deposit sludge, which interferes with heat-transfer in transformers and turbines and also causes plugging of oil feed lines in lubricating systems. Sufficient acid bodies may also be formed to cause reduction in the dielectric strength of these oils.

Solvent-refined oils are those which have been prepared by treatment with selective solvents such as chlorex, phenol, furfural, etc. These oils are similar to moderately acid-refined oils in that metal catalysts such as copper accelerate their oxidation and in that such oxidation is concurrent with substantial color-depreciation and sludge-formation. In general, acid-formation is greater than with moderately acid-refined oils but much less than with highly refined oils. Sludge- and acid-formation lower their value for many purposes, such as those mentioned previously: electrical insulation, lubrication, etc. Solvent-refined oils have found extensive use as lubricants for internal combustion engines because of their high viscosity index, but under the conditions of use encountered in crank cases such oils develop constituents which are corrosive toward certain metal bearings such as the cadmium-silver bearings, etc., which are sometimes used.

It is to be understood that the foregoing classification of oils as "highly refined," "moderately refined," and "solvent-refined" is not to be considered as in any way limiting the scope of this invention, for there can exist oils whose refining 40 blending has been such as to make them intermediate in properties between the foregoing types. Briefly, response to inhibitors may be said to depend entirely upon the type of oxidation and end-products of oxidation of an oil, which in turn depends largely upon the degree of refining this oil has had. Further, the degree of refining required to produce these types of oils varies with the crude source so that any one refining procedure may produce either a highly refined oil or a moderately refined oil, depending upon the crude source. Pennsylvania type oils, for ex-

ample, require much less refining to produce highly refined oils than the Coastal type oils.

Various types of compounds and reaction products have been proposed for use as stabilizers or oxidation-inhibitors for viscous mineral oil fractions. Apparently, the action of these inhibitors is catalytic, and their development is therefore influenced to a great extent by the oxidizable constituents remaining in the oil after a particular refining treatment. Certain inhibitors may be effective to stabilize a mineral oil against sludge-formation and may be ineffective upon acid-formation. Such inhibitors may retard acid-formation in a moderately refined oil but may be totally ineffective in retarding acid-formation in a highly refined oil. Thus, the action of most oxidation-inhibitors is selective, and many such inhibitors are not comprehensive in action so as to stabilize a mineral oil against all of the deleterious effects of oxidation.

As aforesaid, this invention has to do with a novel class of reaction products which has been found to be highly effective as stabilizers for viscous mineral oils refined by any of the methods known to the art and described herein.

This invention is predicated upon the discovery that the reaction products of a dichlor alkyl ether with a primary or secondary aromatic amine are highly effective in small amounts as stabilizers of viscous mineral oils. The amines contemplated herein for reaction with the dichlor alkyl ethers may be represented by the general formula.



wherein R represents an aromatic hydrocarbon radical and R' is selected from the group consisting of hydrogen, aliphatic radicals, and aromatic radicals. It is to be understood that the term "aromatic hydrocarbon radical" as used herein is inclusive of aromatic hydrocarbon radicals having alkyl or aryl substituents; also, that the term "aliphatic radicals" is inclusive of aliphatic radicals having aryl substituents.

More specifically, the reaction products contemplated herein are those formed by reaction of one mol equivalent of a dichlor alkyl ether with at least two, and preferably four, mol equivalents of an aromatic amine of the aforesaid type. Such reaction products are much more effective as stabilizers of viscous mineral oils than are those formed when a lower ratio of reactants is used. In some instances, as when equimolecular proportions of an amine and ether are used, reaction products characterized by a heterocyclic structure are formed. Certain reaction products of this latter type are not effective stabilizers—as, for example, when equimolecular proportions of aniline and beta, beta' dichlor diethyl ether are used, some phenyl morpholine is formed. This compound has been found to be of a lower degree of effectiveness than reaction products of the same reactants obtained by use of at least two, and preferably four, mol equivalents of the amine and one of the ether. These reaction products are viscous oils consisting apparently of mixtures of various constituents; and although they probably contain some diaryl amino-substituted alkyl ethers, their exact composition is uncertain, they are therefore identified and defined herein as reaction products.

Typical reaction products contemplated by this invention are those formed by reaction of dichlor

alkyl mono- and poly-ethers with aromatic amines of the aforesaid type. By the term "mono-ether" is meant an ether characterized by one ethereal oxygen atom, such as



Representative dichlor alkyl mono-ethers which may be used to form the typical reaction products of the class described herein are: dichlor dimethyl ether; beta, beta' dichlor diethyl ether; alpha, beta' dichlor diethyl ether; gamma, gamma' dichlor dipropyl ether; beta, beta' dichlor di-isopropyl ether, etc.

Similarly, the term "poly-ether" is used herein to describe ethers characterized by more than one ethereal oxygen atom, such as



wherein R'' represents an aliphatic radical. Typical dichlor alkyl poly-ethers which may be used for the purposes of this invention are: dichlor triglycol; dichlor tetraglycol, etc.

As aforesaid, the reaction products contemplated herein are obtained by the reaction of a dichlor alkyl (mono- or poly-) ether with a primary or secondary aromatic amine. The primary aromatic amines are characterized by the general formula.



wherein R represents an aromatic hydrocarbon radical and R' is hydrogen. Typical of these primary amines are: aniline, toluidine, xylidine, alpha-naphthylamine, beta-naphthylamine, etc.

The secondary aromatic amines contemplated herein are represented by the general formula.



wherein R represents an aromatic hydrocarbon radical and R' is selected from the group consisting of aliphatic radicals and aromatic radicals as heretofore described. Typical secondary aromatic amines which may serve the purposes of this invention are N-methyl aniline, N-ethyl aniline, N-propyl aniline, N-butyl aniline, N-amyl aniline, N-phenylaniline (diphenylamine), N-ethyl alpha-naphthylamine, N-phenyl alpha-naphthylamine, N-phenyl-beta-naphthylamine, etc.

The general method of preparation of these novel stabilizers consists of heating one molecular proportion of the dichlor alkyl ether with at least two, and preferably with at least four, molecular proportions of the aromatic amine for several hours, treating the mixture with alkali to neutralize any amine hydrochloride formed, and then steam-distilling it to remove unreacted amine and ether. The residual oil is the new stabilizer, which may or may not be further purified. The following typical examples illustrate in detail the preparation of several of the contemplated reaction products:

#### EXAMPLE ONE

*Ethyl aniline-beta, beta' dichlor diethyl ether reaction product:*

96.8 grams (0.8 mol) of ethyl aniline and 28.6 grams (0.2 mol) of beta, beta' dichlor diethyl

ether were heated on a steam bath for 26 hours. The viscous liquid was treated with 200 cc. of a 10 per cent solution of sodium hydroxide and steam-distilled to remove excess reactants. The residue was dissolved in benzene, filtered, solvent-distilled off, and the oil remaining was "topped" to a pot temperature of 210° C. at 2 mm. pressure. The reaction product was a dark-colored viscous oil.

EXAMPLE Two

*Ethyl aniline-dichlor di-isopropyl ether reaction product:*

96.8 grams (0.8 mol) of ethyl aniline and 34 grams (0.2 mol) of dichlor di-isopropyl ether were refluxed for 9 hours. The mixture was treated with 200 cc. of a 12.5 per cent solution of sodium hydroxide and steam-distilled to remove unreacted aniline and dichlor di-isopropyl ether. The residue was dissolved in benzene, filtered, dried, and the solvent evaporated off. The product was a viscous oil.

EXAMPLE THREE

*Aniline-dichlor triglycol ( $ClH_4C_2OC_2H_4OC_2H_4Cl$ ) reaction product:*

74.4 grams (0.8 mol) of aniline and 37.5 grams (0.2 mol) of dichlor diglycol were heated to approximately 200° C. for 8 hours. After the mixture was cooled, 200 cc. of a 12.5 per cent solution of sodium hydroxide were added thereto, and it was steam-distilled to remove unreacted aniline. The residue was taken up in benzene, washed with water, dried, and the solvent evaporated off. The reaction product was a viscous oil.

EXAMPLE FOUR

*Ethyl aniline-dichlor tetraglycol ( $ClH_4C_2OC_2H_4OC_2H_4OC_2H_4Cl$ ) reaction product:*

97 grams (approximately 0.8 mol) of ethyl aniline and 46 grams (0.2 mol) of dichlor tetraglycol were reacted as given in Example Three above. This gave an HCl-soluble viscous oil.

The following tests and results thereof illustrate the effectiveness of the class of reaction products and certain specific members within the class contemplated herein as antioxidants for viscous mineral oil fractions.

TEST No. I

*Oils highly refined with sulfuric acid*

The oil described below and blends thereof were subjected to the modified German tar test. Such a test involves heating a 150-gram sample of the oil at a temperature of 120° C. while bubbling oxygen gas through the oil for a period of 70 hours. The acidic oxidation products formed were then determined by titrating with alcoholic potash. Results for the oil and for the oil blends containing typical reaction products contemplated herein are given in Table I below in terms of neutralization numbers (N. N.), such numbers representing the acidity of the oil at the end of the test.

The oil used in this test was a highly refined oil suitable for use in transformers which had been prepared by treating a Coastal distillate with 40 pounds of 98 per cent sulfuric acid and 180 pounds of 103 per cent oleum per barrel, followed by a clay percolation. It had a specific gravity of 0.871, a flash point of 310° F., and a Saybolt Universal viscosity of 69 seconds at 100° F.

In Table I below and in the following tables, the "addition agent" is identified by the reactants used in preparing the reaction product tested. For example, "aniline-beta, beta' dichlor diethyl ether" indicates the product obtained by reacting these two compounds according to the procedure outlined above.

TABLE I

| 10 | Agent added                                     | Percent used | N. N. value |
|----|-------------------------------------------------|--------------|-------------|
|    | None                                            |              | 25.00       |
| 15 | Aniline-beta, beta' dichlor diethyl ether       | 0.10         | 0.02        |
|    | Ethyl aniline-beta, beta' dichlor diethyl ether | 0.10         | 0.0         |
|    | Aniline-dichlor di-isopropyl ether              | 0.10         | 0.01        |
|    | Aniline-dichlor triglycol                       | 0.10         | 0.0         |
|    | Ethyl aniline-dichlor triglycol                 | 0.10         | 0.0         |
|    | Ethyl aniline-dichlor tetraglycol               | 0.10         | 0.03        |

TEST No. 11

*Oils moderately refined with sulfuric acid*

A mixed Mid-Continent and Coastal distillate had been refined by treatment with 70 pounds of 98 per cent sulfuric acid per barrel, neutralized, washed, and percolated through clay. It had a specific gravity of 0.879, a flash point of 385° F., and a Saybolt Universal viscosity of 152 seconds at 100° F. It is an oil suitable for use in turbines.

This oil and blends thereof containing typical reaction products of the type contemplated herein were tested as follows:

Twenty-five cc. samples of the oil (or the oil blend) were heated to 200° F. with 5 liters of air per hour bubbling through them. Twenty-four inches of No. 18 gauge copper wire and 1 gram of iron granules were added to each sample. Also, 2 cc. of distilled water were added each day. The samples were tested for acidity (N. N.), color, and sludge after varying periods of time. Results are given in Table II below.

TABLE II

| 45 | Agent added                                     | Per cent used | Time, hours         | N. N.               | Lev. color      | Sludge, mg./25 cc. |
|----|-------------------------------------------------|---------------|---------------------|---------------------|-----------------|--------------------|
|    | None                                            |               | { 168<br>240<br>336 | 0.99<br>2.5<br>16.0 | 2<br>110<br>400 | 17<br>246<br>1,282 |
| 50 | Aniline-beta, beta' dichlor diethyl ether       | 0.10          | { 164<br>356        | 0.27<br>6.1         | 7<br>95         | 4<br>336           |
|    | Ethyl aniline-beta, beta' dichlor diethyl ether | 0.10          | { 167<br>672        | 0.01<br>2.8         | 2<br>75         | 40<br>133          |
| 55 | Aniline-dichlor di-isopropyl ether              | 0.10          | { 166<br>497        | 0.01<br>1.1         | 1<br>14         | 10<br>7            |
|    | Ethyl aniline-dichlor di-isopropyl ether        | 0.10          | { 161<br>497        | 0.01<br>0.0         | 1<br>2          | 5<br>16            |
| 60 | Aniline-dichlor triglycol                       | 0.10          | { 1,505<br>497      | 5.2<br>5.8          | 130<br>110      | 326<br>165         |
|    | Ethyl aniline-dichlor tetraglycol               | 0.10          | { 166<br>503        | 0.09<br>2.6         | 4<br>100        | 4<br>111           |

TEST No. III

*Oils refined by means of solvents*

The oil used in this test was a distillate from a Rodessa crude which had been refined with furfural, dewaxed, and filtered. The finished stock had a Saybolt Universal viscosity of 151 seconds at 100° F. This oil and blends thereof were tested by the method described in Test No. II above. The results are set forth in Table III below.

TABLE III

| Agent added                                     | Per cent used | Time, hours | N. N. | Lov. color | Sludge, mg./25 cc. |
|-------------------------------------------------|---------------|-------------|-------|------------|--------------------|
| None                                            |               | 92          | 0.91  | 9          | 33                 |
| Aniline-beta, beta' dichlor diethyl ether       | 0.10          | 165         | 20.3  | 320        | 251                |
|                                                 |               | 164         | 0.01  | 1          | 5                  |
|                                                 |               | 500         | 0.08  | 1          | 15                 |
| Ethyl aniline-beta, beta' dichlor diethyl ether | 0.10          | 692         | 3.9   | 13         | 106                |
| Aniline-dichlor di-isopropyl ether              | 0.10          | 167         | 0.06  | 1          | 13                 |
| Ethyl aniline-dichlor di-isopropyl ether        | 0.10          | 359         | 1.0   | 1          | 10                 |
| Ethyl aniline-dichlor triglycol                 | 0.10          | 166         | 0.01  | 1          | 6                  |
| Ethyl aniline-dichlor tetraglycol               | 0.10          | 503         | 0.01  | 1          | 3                  |
|                                                 |               | 161         | 0.01  | 1          | 2                  |
|                                                 |               | 1,505       | 0.01  | 1          | 94                 |
|                                                 |               | 161         | 0.01  | 1          | 2                  |
|                                                 |               | 497         | 0.4   | 4          | 8                  |
|                                                 |               | 161         | 0.9   | 6          | 25                 |

## TEST NO. IV

## Corrosion test

Motor oils, especially those refined by certain solvent-extraction methods, tend to oxidize when submitted to high temperature and to form products that are corrosive to metal bearings. This corrosive action may be quite severe with certain bearings, such as those having the corrosion-susceptibility of cadmium-silver alloys; and it may cause their failure within a comparatively short time. The following test was used to determine the corrosive action of a motor oil on an automobile connecting-rod bearing.

The oil used consisted of Pennsylvania neutral and residuum stocks separately refined by means of chlorex and then blended to give an S. A. E. 20 motor oil with a specific gravity of 0.872, a flash point of 435° F., and a Saybolt Universal viscosity of 318 seconds at 100° F. The oil was tested by adding a section of a bearing containing a cadmium-silver alloy surface and weighing about 6 grams and heating it to 175° C. for 22 hours while a stream of air was bubbled against the surface of the bearing. The loss in weight of the bearing during this treatment measures the amount of corrosion that has taken place. A sample of the oil containing a stabilizer was run at the same time as a sample of the straight oil, and the loss in weight of the bearing section in the inhibited oil could thus be compared directly with the loss of the section in the uninhibited oil. The results obtained in this test are set forth in Table IV below.

TABLE IV

| Agent added                               | Per cent used | Mg. loss in weight |             |
|-------------------------------------------|---------------|--------------------|-------------|
|                                           |               | Inhibited          | Uninhibited |
| Aniline-beta, beta' dichlor diethyl ether | 0.25          | 0                  | 31          |
| Ethyl aniline-dichlor di-isopropyl ether  | 0.25          | 0                  | 32          |

From the foregoing test results it will be observed that the reaction products contemplated herein are highly effective to stabilize viscous petroleum oil fractions against the normal deteriorating effects of oxidation as manifested by development of acidity, color and sludge, irrespective of the refining treatment which the oil has received; and further that certain of these reaction products are highly effective to retard the corrosive action encountered when certain oils are used in connection with normally corrosive alloy bearings. The quantity of reaction product used to inhibit the deleterious effects of

oxidation upon the oil may be varied depending upon the character of the oil and the severity of the conditions to which it is to be exposed, but in general it appears that the desired results may be obtained with an amount varying from 0.01 per cent to 1.00 per cent.

It is to be understood that while I have herein described in detail certain typical reaction procedures and several specific reactants which may be employed in synthesizing the reaction products contemplated herein, the invention is not confined to these specific procedural details or reactants but includes within its scope such changes and modifications as fairly come within the spirit of the appended claims.

I claim:

1. An improved mineral oil composition comprising a viscous mineral oil fraction and in admixture therewith a minor proportion of a reaction product obtained by reaction of a dichlor alkyl ether and an aromatic amine represented by the general formula



wherein R represents an aromatic hydrocarbon radical and R' is selected from the group consisting of hydrogen, aliphatic radicals and aromatic radicals, said product being present in an amount sufficient to inhibit the deleterious effects of oxidation upon the oil.

2. An improved mineral oil composition comprising a viscous mineral oil fraction and in admixture therewith a minor proportion of a reaction product obtained by reaction of one mol equivalent of a dichlor alkyl ether and at least two mol equivalents of an aromatic amine represented by the general formula



wherein R represents an aromatic hydrocarbon radical and R' is selected from the group consisting of hydrogen, aliphatic radicals and aromatic radicals, said product being present in an amount sufficient to inhibit the deleterious effects of oxidation upon the oil.

3. An improved mineral oil composition comprising a viscous mineral oil fraction and in admixture therewith a reaction product obtained by reaction of one mol equivalent of a dichlor alkyl ether and at least two mol equivalents of an aromatic amine represented by the general formula



wherein R represents an aromatic hydrocarbon radical, and R' is selected from the group consisting of hydrogen, aliphatic radicals, and aromatic radicals, said product being present in an amount of from about 0.01 per cent to about 1.00 per cent.

4. An improved mineral oil composition comprising a viscous mineral oil fraction and in admixture therewith a minor proportion of a reaction product obtained by reaction of one mol equivalent of a dichlor alkyl monoether and at least two mol equivalents of an aromatic amine represented by the general formula



wherein R represents an aromatic hydrocarbon radical and R' is selected from the group consisting of hydrogen, aliphatic radicals, and aromatic radicals, said product being present in an amount sufficient to inhibit the deleterious effects of oxidation upon the oil.

5. An improved mineral oil composition comprising a viscous mineral oil fraction and in admixture therewith a minor proportion of a reaction product obtained by reaction of one mol equivalent of beta, beta' dichlor diethyl ether and at least two mol equivalents of an aromatic amine represented by the general formula



wherein R represents an aromatic hydrocarbon radical and R' is selected from the group consisting of hydrogen, aliphatic radicals, and aromatic radicals, said product being present in an amount sufficient to inhibit the deleterious effects of oxidation upon the oil.

6. An improved mineral oil composition comprising a viscous mineral oil fraction and in admixture therewith a minor proportion of a reaction product obtained by reaction of one mol equivalent of a dichlor alkyl polyether and at least two mol equivalents of an aromatic amine represented by the general formula



wherein R represents an aromatic hydrocarbon radical and R' is selected from the group consisting of hydrogen, aliphatic radicals, and aromatic radicals, said product being present in an amount sufficient to inhibit the deleterious effects of oxidation upon the oil.

7. An improved mineral oil fraction comprising a viscous mineral oil fraction and in admixture therewith a minor proportion of a reaction product obtained by reaction of one mol equivalent of a dichlor triglycol and at least two mol equivalents of an aromatic amine represented by the general formula



wherein R represents an aromatic hydrocarbon radical and R' is selected from the group consisting of hydrogen, aliphatic radicals, and aromatic radicals, said product being present in an amount sufficient to inhibit the deleterious effects of oxidation upon the oil.

8. An improved mineral oil composition comprising a viscous mineral oil fraction and in admixture therewith a minor proportion of a reaction product obtained by reaction of one mol equivalent of a dichlor alkyl ether and at least two mol equivalents of a primary aromatic amine, said product being present in an amount sufficient to inhibit the deleterious effects of oxidation upon the oil.

9. An improved mineral oil composition comprising a viscous mineral oil fraction and in admixture therewith a minor proportion of a reaction product obtained by reaction of one mol equivalent of a dichlor alkyl ether and at least two mol equivalents of aniline, said product being present in an amount sufficient to inhibit the deleterious effects of oxidation upon the oil.

10. An improved mineral oil composition comprising a viscous mineral oil fraction and in admixture therewith a reaction product obtained by reaction of one mol equivalent of a dichlor alkyl ether and at least two mol equivalents of aniline, said product being present in an amount of from about 0.01 per cent to about 1.0 per cent.

11. An improved mineral oil composition comprising a viscous mineral oil fraction and in admixture therewith a minor proportion of a reaction product obtained by reaction of one mol equivalent of a dichlor alkyl ether and at least two mol equivalents of a secondary aromatic amine, said product being present in an amount sufficient to inhibit the deleterious effects of oxidation upon the oil.

12. An improved mineral oil composition comprising a viscous mineral oil fraction and in admixture therewith a minor proportion of a reaction product obtained by reaction of one mol equivalent of a dichlor alkyl ether and at least two mol equivalents of ethyl aniline, said product being present in an amount sufficient to inhibit the deleterious effects of oxidation upon the oil.

13. An improved mineral oil composition comprising a viscous mineral oil fraction and in admixture therewith a reaction product obtained by reaction of one mol equivalent of a dichlor alkyl ether and at least two mol equivalents of ethyl aniline, said product being present in an amount of from about 0.01 per cent to about 1.00 per cent.

14. An improved mineral oil composition comprising a viscous mineral oil fraction and in admixture therewith a minor proportion of a reaction product obtained by reaction of one mol equivalent of a dichlor alkyl ether selected from the group consisting of dichlor dimethyl ether; beta, beta' dichlor diethyl ether; alpha, beta' dichlor diethyl ether; gamma gamma' dichlor di-propyl ether; beta, beta' dichlor di-isopropyl ether; dichlor triglycol; and dichlor tetraglycol, and at least two mol equivalents of an aromatic amine represented by the general formula



wherein R represents an aromatic hydrocarbon radical and R' is selected from the group consisting of hydrogen, aliphatic radicals, and aromatic radicals, said product being present in an amount sufficient to inhibit the deleterious effects of oxidation upon the oil.

15. An improved mineral oil composition comprising a viscous mineral oil fraction and in admixture therewith a minor proportion of a reaction product obtained by reaction of one mol equivalent of a dichlor alkyl ether selected from the group consisting of dichlor dimethyl ether; beta, beta' dichlor diethyl ether; alpha, beta' dichlor diethyl ether; gamma, gamma' dichlor di-propyl ether; beta, beta' dichlor di-isopropyl ether; dichlor triglycol; and dichlor tetraglycol, and at least two mol equivalents of a primary aromatic amine, said product being present in an amount sufficient to inhibit the deleterious effects of oxidation upon the oil.

16. An improved mineral oil composition comprising a viscous mineral oil fraction and in admixture therewith a minor proportion of a reaction product obtained by reaction of one mol equivalent of a dichlor alkyl ether selected from the group consisting of dichlor dimethyl ether; beta, beta' dichlor diethyl ether; alpha, beta' di-

chlor diethyl ether; gamma, gamma' dichlor di-propyl ether; beta, beta' dichlor di-isopropyl ether; dichlor triglycol; and dichlor tetraglycol, and at least two mol equivalents of aniline, said product being present in an amount sufficient to inhibit the deleterious effects of oxidation upon the oil.

17. An improved mineral oil composition comprising a viscous mineral oil fraction and in admixture therewith a minor proportion of a reaction product obtained by reaction of one mol equivalent of a dichlor alkyl ether selected from the group consisting of dichlor dimethyl ether; beta, beta' dichlor diethyl ether; alpha, beta' dichlor diethyl ether; gamma, gamma' dichlor di-propyl ether; beta, beta' dichlor di-isopropyl ether; dichlor triglycol; and dichlor tetraglycol; and at least two mol equivalents of a secondary

aromatic amine, said product being present in an amount sufficient to inhibit the deleterious effects of oxidation upon the oil.

18. An improved mineral oil composition comprising a viscous mineral oil fraction and in admixture therewith a minor proportion of a reaction product obtained by reaction of one mol equivalent of a dichlor alkyl ether selected from the group consisting of dichlor dimethyl ether; beta, beta' dichlor diethyl ether; alpha, beta' dichlor diethyl ether; gamma, gamma' dichlor di-propyl ether; beta, beta' dichlor di-isopropyl ether; dichlor triglycol; and dichlor tetraglycol; and at least two mol equivalents of ethyl aniline, said product being present in an amount sufficient to inhibit the deleterious effects of oxidation upon the oil.

EVERETT W. FULLER.